

Patented Dec. 7, 1926.

1,609,798

## UNITED STATES PATENT OFFICE.

GUST A. DANIELSON, OF LOS ANGELES, CALIFORNIA.

### LEATHER-WATERPROOFING COMPOSITION.

No Drawing.

Application filed July 18, 1923. Serial No. 652,449.

The object of my invention is the production of a water proof composition, which when applied to the surface of leather acts as a preservative for the leather and renders it absolutely water proof. My composition consists of a mixture of tallow, beeswax, neat's-foot oil, rosin, turpentine, and paraffine. In preparing the composition, I prefer to use the ingredients in about the following proportions:

Tallow, 1 pound; beeswax,  $\frac{3}{4}$  pound; neat's-foot oil, 1 quart; rosin, 1 ounce; turpentine,  $\frac{1}{2}$  pint; paraffine, 1 ounce.

Good results may be obtained, however, when the ingredients are varied in that more tallow, and less rosin can be used, but a higher priced product would be the result. These ingredients are mixed and form a paste of such consistency as to enable it to be

plastered over the surface to be protected. It may be applied in one or more coats or layers in the ordinary manner according to the nature of the article and the amount of protection required, by allowing the first coat or layer to soak into the leather and dry before applying the second coat or layer.

My composition is light and water proof and penetrates the leather without cracking when it dries.

I claim:

A composition formed of one pound of tallow, one fourth pound of beeswax, one quart of neat's-foot oil, one ounce of rosin, one half pint of turpentine and one ounce of paraffine, for the purpose specified.

Dated at Los Angeles, California, this 12th day of July, 1923.

GUST A. DANIELSON.